

1

3,825,544

## 7 PIPERAZINOFLUORANS

Mutsuo Terayama and Kenji Yamamoto, Osaka, Japan, assignors to Yamamoto Kagaku Gosei Kabushiki Kaisha

No Drawing. Filed Dec. 15, 1971, Ser. No. 208,432

Claims priority, application Japan, Dec. 15, 1970,

45/112,052

Int. Cl. C07d 51/70

U.S. CL. 260—268 PC

5 Claims

### ABSTRACT OF THE DISCLOSURE

An excellent pressure sensitive copying sheet is provided by applying as a color former certain encapsulated fluoran compounds, i.e. fluoran compounds linking in the 7-position with at least one of the two nitrogen atoms in a piperazine ring and having a dialkylamino group in the 3-position to either a single sheet or to the upper leaf of a pressure sensitive paper. The color former is soluble in aromatic solvents and also has excellent light fastness.

### BACKGROUND OF THE INVENTION

Basically, pressure sensitive copying sheet consists of two sheets of paper, an upper leaf and a lower leaf, the lower surface of the upper leaf being coated with minute capsules containing a color reactive achromatic substance (hereinafter called a "color former") dissolved in a low volatile solvent and the upper surface of the lower leaf being coated with a solid acid, such as acid clay, zeolite, bentonite, attapulgite and phenolic compound, etc. When the lower surface of the upper leaf and upper surface of the lower leaf are put together and pressure is applied to the upper surface of the upper leaf by handwriting or typing, the capsules under pressure are broken and the color former contained therein is adsorbed by the solid acid on the upper surface of the lower leaf to develop a color, and thereby the object of copying is attained.

There is also a type of pressure sensitive copying sheet having a mechanism to develop a color when a regional pressure is exerted upon a sheet of paper holding capsules, which contain a color former, and a solid acid on or within it. However, such type is quite similar to the first-mentioned pressure sensitive copying paper (consisting of two sheets of paper, an upper and lower leaf) with respect to the mechanism of developing a color, and thus the same color former can be used for both types. And any of the above-mentioned facts belongs to the prior-known arts.

Conventionally, a number of compounds have been known to be useful as the color former, such as lactones, i.e. crystal violet lactone and malachite green lactone; thiazine compounds, i.e. benzoyl leucomethylene blue; and other leucoauramine and spiropyran compounds, and others.

In most of the pressure sensitive copying sheets now in practical use, crystal violet lactone and benzoyl leucomethylene blue, both of which develop a blue color, are used as the main color former. But the blue image due to these color formers is not suitable for recopying by Xerox or diazo system. It has therefore been hoped for to find out some solution for this defect. This defect can be solved by obtaining a black image in two ways: (1) to employ a black color former, or (2) to employ two or more color formers in combination for synthesizing a black image.

### SUMMARY

In accordance with the invention, an excellent pressure sensitive copying paper can be obtained by using a new and novel color former which is very advantageous in obtaining a black image, offering superiority not only in the speed of color development, the shade, and the light

2

resistance of the color developed, and the solubility but also in the simplicity of the manufacturing method and the low cost. The new and novel color former used in the present invention all develop into either black or red. One which develops into black can be used alone, while the other which develops into red can advantageously produce a highly stabilized black image when mixed with one other color former which develops into green (for example, 3-diethylamino-7-benzylaminofluoran (see Canadian Pat. No. 814,948)).

The color former used in the present invention can be represented by the following general formulae (I) and (II).



(I)

wherein R<sub>1</sub>, R<sub>2</sub> and R<sub>5</sub> represent methyl or ethyl, and R<sub>3</sub> and R<sub>4</sub> represent hydrogen, methyl group, or halogen.



(II)

wherein R<sub>1</sub>, R<sub>2</sub>, R<sub>3</sub> and R<sub>4</sub> are the same as in the general formula (I).

That is to say, we have found that the fluoran compounds linking in the 7-position with at least one of the two nitrogen atoms in a piperazine ring and having a dialkylamino group in the 3-position can become the black and red color formers which are distinguished in all of the color developing speed, the shade and the light resistance of the color developed and the solubility and that they can be readily synthesized by the process shown by the following reaction formula.





wherein R<sub>1</sub>, R<sub>2</sub>, R<sub>3</sub>, R<sub>4</sub> and R<sub>5</sub> are the same as in the general formula (I).

(III) can be prepared with much ease by the following reaction formula (See Beilstein, Hauptwerk, vol. 23, p. 11.)



#### DETAILED DESCRIPTION

The following are typical examples of the novel color former.

##### 3-Diethylamino-7-(N'-paramethoxyphenyl)piperazinofluoran (IV)



This compound (IV) is a white crystal obtained by condensing 2 parts of ortho-(4-diethylamino-2-hydroxybenzoyl)benzoic acid (V) and 3 parts of N,N'-di(paramethoxyphenyl)piperazine (VI) in concentrated sulfuric acid and having a melting point of 237 to 240° C. It has the characteristics which are highly advantageous for the preparation of the pressure sensitive copying sheet, such as the rapid development into a black or blackish red color in the presence of a solid acid, and the excellent light resistance of the color developed as well as the high solubility in the solvent.



The compound (VI) can be readily obtained by refluxing under heat paraanisidine and dibromoethane in the presence of sodium carbonate.



(VII) is a white crystal obtained by condensing 4 parts of (V) and 3 parts of (VI) in concentrated sulfuric acid and having a melting point of 265 to 270° C. It also has the characteristics which are highly advantageous for the preparation of the pressure sensitive copying sheet, such as the rapid development into a black or blackish red color in the presence of solid acid, and the excellent light resistance of the color developed as well as the high solubility in the solvent.



(VIII) is a white crystal obtained by condensing 2 parts of (V) and 1 part of (VI) in concentrated sulfuric acid and having a melting point of 210 to 215° C. This also rapidly develops into a dark red color in the presence of a solid acid, has an excellent light resistance after developing into a color, and dissolves well in the solvent.

The present invention is further illustrated by the following examples.

#### Example 1

60 g. of gelatin and 60 g. of gum arabic were dissolved in 50 ml. of water of 40° C. On the other hand, 4 g. of 3-diethylamino-7-(N'-paramethoxyphenyl)piperazinofluoran (IV) was dissolved in 120 g. of diphenyl chloride, and then this solution was added to the above-mentioned aqueous solution of gelatin and gum arabic and perfectly dispersed into an emulsion by a homo-mixer. Water of 50° C. was added until its volume became 2,000 ml. in total, followed by 90 ml. of 10 percent acetic acid. While stirring, water of 50° C. was further added until the total weight became 4 kg., and the stirring was continued for a period of an hour. While still stirring, the solution was cooled down to below 10° C. with ice water, and 10 percent caustic soda was added until a pH of 9, was reached, and gradually returned to room temperature. The product was applied onto the lower surface of the upper leaf and dried. On the other hand, a solid acid such as acid clay or phenolic compounds, etc. was applied onto the upper surface of the lower leaf.

When copying was carried out with the upper and lower leaves thus prepared, a black or blackish red image rapidly developed, which showed an excellent light resistance.

#### Example 2

4 g. of N,N'-bis(3'-diethylaminofluoranyl)piperazine (VII) was dissolved in 120 g. of diphenyl chloride, which solution was then treated in the same way as in Example 1 to obtain the pressure sensitive copying sheet.

When copying was carried out with this copying sheet, a black or blackish red image rapidly developed, which showed an excellent light resistance.

#### Example 3

1.0 g. of N,N'-bis(3'-diethylamino-6'-methylfluoranyl)piperazine (VIII) and 2.5 g. of 3-diethylamino-7-benzylaminofluoran (See Canadian Pat. No. 814,948) were dissolved in 120 g. of diphenyl chloride, which solution was then treated in the same way as in Example 1 to obtain the pressure sensitive copying sheet. When copying was carried out with this copying sheet, a black image rapidly developed, which showed an excellent light resistance.

## 5

## Example 4

4 g. of N,N'-bis(3'-diethylaminofluoranyl)piperazine (VII) was dissolved in 120 g. of diphenyl chloride. By treating this in the same way as in Example 1, an aqueous dispersion of minute capsules was obtained. This was sprayed and dried into a powder of minute capsules, which was mixed with and dispersed in a 4 percent xylene solution of p-phenylphenol formaldehyde condensate. And this dispersed solution was applied onto a sheet of paper and dried. When a regional pressure was exerted on this coated sheet of paper, it immediately developed a black image, which showed an excellent light resistance.

## Example 5

4 g. of N,N'-bis(3'-diethylamino-6'-methylfluoranyl)piperazine (VIII) was dissolved in 120 g. of diphenyl chloride.

By treating this solution in the same way as in Example 1, an aqueous dispersion of minute capsules was obtained. This was mixed with 8 g. of fine powder of p-phenylphenol formaldehyde condensate to disperse the latter therein, and 40 g. of pulp was further added thereto. Then the dispersion was diluted with water until the final solid content became 0.5 percent. Then the product was run onto a Fourdrinier screen to be made into a sheet of paper. When a regional pressure was exerted on this sheet of paper, it immediately developed a black image with an excellent light resistance.

Although diphenyl chloride was used as a solvent in the foregoing examples, the same pressure sensitive copying paper can be obtained without problem with the use of other aromatic solvent. These aromatic solvents of low volatility include lower alkyl diphenyls, such as methyl-, ethyl- and propyl diphenyl, and higher alkyl benzenes, such as dodecyl-, decyl- and octyl benzene, having a boiling point of above 150 C. If the boiling point of the solvent is at least 150 C., it has sufficient low volatility according to the invention.

The solid acid functions as an electron acceptive adsorbent. In place of those used in the previous examples zeolite, bentonite, attapulgite and Silton® (manufactured and sold by Mizusawa Chemical Company Ltd.) can be used with excellent results.

What is claimed is:

1. A fluoran of the formula

5

10

15

20

25

30

35

40

45



wherein each of R<sub>1</sub> and R<sub>2</sub> is methyl or ethyl; each of R<sub>3</sub> and R<sub>4</sub> is hydrogen, methyl or halogen; and A is either



wherein R<sub>5</sub> is methyl or ethyl; and R<sub>1</sub>, R<sub>2</sub>, R<sub>3</sub> and R<sub>4</sub> are as defined above.

2. A fluoran of claim 1, wherein R<sub>3</sub> and R<sub>4</sub> are hydrogen or methyl.

3. Fluoran compound of claim 1 which is 3-diethylamino-7-(N'-paramethoxyphenyl)piperazinofluoran.

4. Fluoran compound of claim 1 which is N,N'-bis(3'-diethylaminofluoranyl)piperazine.

5. Fluoran compound of claim 1 which is N,N'-bis(3'-diethylamino-6'-methylfluoranyl)piperazine.

## References Cited

## UNITED STATES PATENTS

3,442,908 5/1969 Orita ----- 260—335

DONALD G. DAUS, Primary Examiner

## U.S. CL. X.R.

117—36.2; 260—268 BI, 268 PA, 518 R

UNITED STATES PATENT OFFICE  
CERTIFICATE OF CORRECTION

Patent No. 3,825,544 Dated July 23, 1974

Inventor(s) Mutsuo Terayama and Kenji Yamamoto

It is certified that error appears in the above-identified patent and that said Letters Patent are hereby corrected as shown below:

Column 2, Formula I:



Column 2, Formula II: The formula should read as follows:



Column 4, line 68: "N,N-bis" should read --N,N'-bis--.

UNITED STATES PATENT OFFICE  
CERTIFICATE OF CORRECTION

Patent No. 3,825,544 Dated July 23, 1974

Inventor(s) Mutsuo Terayama and Kenji Yamamoto Page 2

It is certified that error appears in the above-identified patent and that said Letters Patent are hereby corrected as shown below:

Column 6, line 20: The second formula should read as follows:



Signed and sealed this 6th day of May 1975.

(SEAL)

Attest:

RUTH C. MASON  
Attesting Officer

C. MARSHALL DANN  
Commissioner of Patents  
and Trademarks